# EUROPEAN PATENT SPECIFICATION

(11) **EP 0 034 057 B1**
(45) Date of publication and mention of the grant of the patent: **15.08.1984**
(21) Application number: 81300509.7
(22) Date of filing: 06.02.1981
(51) Int. Cl.: C21D 9/50, C21D 3/06, C21D 11/00

(54) **Method for postweld heat treatment**
Wärmebehandlungsverfahren für Schweissstellen
Procédé de traitement thermique de joints soudés

(30) Priority: 09.02.1980 JP 14997/80
(43) Date of publication of application: 19.08.1981
(73) Proprietor: KABUSHIKI KAISHA KOBE SEIKO SHO, Kobe 651 (JP)
(72) Inventor: Takahashi, Eiji, 1-chome Hyogo-ken (JP); Iwai, Kenji, 2-chome Suma-ku Kobe (JP)
(74) Representative: Wright, Hugh Ronald

## Description

This invention relates to a method for postweld heat treatment (hereinafter referred to as PWHT) of a welded portion of, for example, a thick base metal, and more particularly to a method for appropriately judging the time point for terminating the PWHT when sufficient of the residual diffusible hydrogen in the welded metal has been dissipated by the afterheating.

There sometimes occurs a problem of cold (or delayed) cracking when welding thick low alloy steels. At present, it is the usual practice to resort to intermediate stress relief annealing to prevent cracking of that sort. However, as seen in disulfurizing reaction towers and coal liquefaction systems, there is a recent distinctive trend in the chemical industries toward larger scale plants, which involve for an increased number of times the intermediate stress relief annealing treatment after welding. Repetitive intermediate stress relief annealing not only gives rise to deteriorations in strength and toughness of the material but also hinders the fabrication process, thus increasing the length of time of the process and the cost of the fabrication.

Under these circumstances, the present inventors have conducted research into multilayer butt welds of thick 2j-Cr-1 Mo steel and A508 Class 3 material and found that: (1) the problematic cracks are mostly transverse cracks in a weld zone, that is to say, in weld metal or in the heat affected zone (HAZ); (2) the cracks are apt to occur immediately beneath the final layer due to the residual stress in the direction of weld line, diffusible hydrogen and hard microstructure, propagating and growing toward the inner and outer surfaces of a plate; and (3) the residual stress remains almost the same independent of the plate thickness but the residual hydrogen decreases upon raising the preheat and interpass temperature at the time of welding, thereby preventing the occurrence of a crack. From these facts, it is deduced that an effective means for preventing cracks is to decrease the diffusible hydrogen concentration in the weld zone.

This situation is also recognised in "Welding Journal" volume 58 no. 52 (February 1979) see in particular page 57 left column, but no rules are given how to determine the critical hydrogen concentration in different circumstances. Therefore the limit for the critical hydrogen concentration was set at such a low level that, independent of welding parameters, cracking could not occur in any case.

Our research was focused on the so-called low temperature PWHT which prevents the cracking by decreasing the diffusible hydrogen concentration in a weld zone by heating the weld zone to a relative low temperature immediately after welding. Since this method is intended to prevent cracking solely through the diminution of the diffusible hydrogen concentration in the weld zone, we sought to clarify the following items before its application.
(1) The relation between the conditions of the welding operation for an actual structure and the hydrogen concentration immediately after welding.
(2) The relation between the variations in the hydrogen concentration during low temperature PWHT and the treating conditions.
(3) The relation between the critical hydrogen concentration at which the possibility of cracking is eliminated and the maximum Vicker's hardness number in the weld zone.

The present inventors clarified the items (1) to (3) by experiments on butt weldments of thick 24Cr-1Mo steel and A508 Class 3 material and furthered their research on the basis of the experimental data. As a result, they succeeded in preventing the cracking by an appropriate PWHT, thereby permitting the omission of an intermediate stress relief annealing step.

More particularly, one aspect of the present invention provides:
a method for the low-temperature PWHT in multilayer welding, comprising the steps of:
   determining the residual hydrogen concentration Co (cc/100 g) directly beneath the final welded layer immediately after completion of welding;
   determining a crack-preventing critical hydrogen concentration Ccr (cc/100 g) to obtain a ratio of Ccr/Co;
   determining the value of a product Dp.tp of a hydrogen diffusivity coefficient Dp (cm²/sec.) during the heat treatment and a holding time tpfsec.) where a currently reached hydrogen concentration C (cc/100 g) become equal to the critical hydrogen concentration Ccr, on the basis of the relation of a ratio C/Co of the current hydrogen concentration Cfcc/100 g) to the residual hydrogen concentration Co and a sum of a parameter τ (cm²) of hydrogen diffusion of the formula given below and the product of Dp-tp;
   measuring the temperature of the heat treatment at a suitable position of the weld;
   terminating the heat treatment at the time point when a time-integrated value of a hydrogen diffusivity coefficient D_{Pi}(cm²/sec.) at the measured temperature exceeds the value of Dp.tp under given conditions wherein,
      PWHT: postweld heat treatment,
      D_{;}: a hydrogen diffusivity coefficient (cm²/sec.) in an arbitrary weld portion during welding each unit layer; and
      tn: time (sec.) required for welding each unit layer, and wherein the critical hydrogen concentration, (Ccr) is related to the Vicker's hardness number, (Hv) such that (Ccr) ranges from 1.96 to 3.88 cc/100 g while (Hv) correspondingly ranges from 300 to 500.

The present invention also provides a method for the low-temperature postweld heat treatment in multilayer welding, comprises the steps of;
obtaining the residual hydrogen concentration (Co)_{D} and (Co)_{H} (cc/100 g) directly beneath the finally welded layer immediately after completion of multilayer welding, where (Co), and (Co)_{H} are for weld metal (deposited metal) and for heat affected zone, respectively;
obtaining the critical hydrogen concentration for prevention of cracking (Ccr)_{D} and (Ccr)_{H} for the weld metal and for the heat affected zone, respectively, which depend upon the maximum residual stress and maximum Vicker's hardness number of microstructure in weld zone;
obtaining the values of (Ccr/Co)_{D} and (Ccr/Co)_{H}, ratio of the critical hydrogen concentration (Ccr)_{D} and [Ccr]_{H} for prevention of cracking both in the weld metal and the heat affected zone to the residual hydrogen concentration [Co] and [C_{O}]_{H};
obtaining the values of [C/Co]_{D} and [C/Co]_{H} for the weld metal and for the heat affected zone, the ratio of the hydrogen concentration in the weld zone [C]ₒ and [C]_{H} which are lessen by the low-temperature postweld heat treatment to the residual hydrogen concentration [Co]_{D} and [Co]_{H};
obtaining the values of [τ + Dₚ·tₚ]_{D} and [τ + Dₚ·tₚ]_{H} for the weld metal and for the heat affected zone where Dp is hydrogen diffusivity coefficient during the postweld heat treatment and tp is the holding time, and _{T} (cm²) is a hydrogen diffusion parameter in a welding operation under given conditions wherein
D, is a hydrogen diffusivity coefficient (cm²/sec.) in an arbitrary weld zone of each unit and tn is the time required for welding each unit layer;
determining a larger value [Dₚ·tₚ] of [Dₚ·tₚ]_{D} or (Dₚ·ₜp]_{H} by comparing those values, as a condition of the postweld heat treatment;
measuring the temperature at a suitable portion of the weld during the postweld heat treatment, and
terminate the heat treatment at a time point when the time integrated value of the hydrogen diffusivity coefficient (Dₚᵢ) (cm2/sec.) at the measured temperature exceeds the value of (D_{P}·t_{P}), and wherein. the critical hydrogen concentrations (Ccr)_{D} and (Ccr)_{H} are related to the Vicker's hardness numbers, (Hv)p and (Hv), respectively such that (Ccr)_{D} and (Ccr)_{H} range from 1.96 to 3.88 cc/100 g while (Hv)_{D} and (Hv)_{H} correspondingly range from 300 to 500.

By the way, when the maximum Vicker's hardness number of the microstructure in the weld metal is higher than that in the Haz, the estimation of above mentioned respective values only for weld metal is sufficient because the hydrogen concentration in HAZ is generally much lower than that in weld metal.

In the method of the present invention, for instance, the first step of observing the value of (co) can be realised by various means or procedures in practical applications. The gist of the invention resides in the above mentioned steps and is not limited to practical procedures employed therefor. The particular procedures developed in the description are given only as typical examples and should not be construed as limiting the present invention. In this regard, it is to be noted that the invention includes all modifications and alterations as encompassed by the appended claims.

The present invention also provides a method for the low-temperature PWHT of a multilayer weld, characterised by the steps of:
determining for a test weld similar to said multilayer weld the residual hydrogen concentration Co (cc/100 g) directly beneath the final welded layer immediately after completion of welding;
determining for the test weld a crack-preventing critical hydrogen concentration Ccr (cc/100 g) to obtain a ratio of Ccr/Co;
determining for the test weld the value of a product D_{P}·tₚ of a hydrogen diffusivity coefficient Dp(cm²/sec.) during the heat treatment and a holiday time tp (sec.) where a currently reached hydrogen concentration C (cc/100 g) becomes equal to the critical hydrogen concentration Ccr, on the basis of the relation of a ratio C/Co of the current hydrogen concentration C(cc/100 g) to the residual hydrogen concentration Co and a sum of a parameter τ (cm2) of hydrogen diffusion of the formula given below and the product of Dp.tp;
measuring for said multilayer weld the temperature of the heat treatment at a suitable position of the weld;
terminating the heat treatment of said multilayer weld at a time point when a time integrated value of the previously determined hydrogen diffusivity coefficient Dpi (cm²/sec.) at the measured temperature exceeds the previously determined value of Dp.tp. wherein,
PWHT: postweld heat treatment,
D,: a hydrogen diffusivity coefficient (cm²/sec.) in an arbitrary weld portion during welding each unit layer; and
tn: time (sec.) required for welding each unit layer, and wherein the critical hydrogen concentration, (Ccr), is related to the Vicker's hardness number, (Hv), such that (Ccr) ranges from 1.96 to 3.88 cc/100 g while (Hv) correspondingly ranges from 300 to 500.

The present invention also provides a method for the low temperature postweld heat treatment of a multilayer weld, characterised by the steps of:
obtaining for a test weld similar to said multilayer weld, the residual hydrogen concentration (Co)_{D} and (C_{O})_{H} (cc/100 g) directly beneath the finally welded layer immediately after completion of multilayer welding, where (Co)_{D} and (Co)_{H} are for weld metal (deposited metal) and for heat affected zone, respectively;
obtaining for the test weld the critical hydrogen concentration for preventing of cracking (Ccr)_{D} and (Ccr)_{H} for the weld metal and for the heat affected zone, respectively, which depend upon the maximum residual stress and maximum Vicker's hardness number of the microstructure in the weld zone;
obtaining for the test weld the values of (Ccr/Co)_{D} and (Ccr/Co)_{H}, the ratio of the critical hydrogen concentration (Ccr)_{D} and (Ccr)_{H} for prevention of cracking both in the weld metal and the heat affected zone to the residual hydrogen concentration (Co)_{D} and (Co)_{H};
obtaining for the test weld the values of (C/Co)_{D} and (C/Co)_{H} for the weld metal and for the heat affected zone, the ratio of the hydrogen concentration (C)_{D} and (C)_{H} which are lessened by the low temperature postweld heat treatment to the residual hydrogen concentration (Co)_{D} and (Co)_{H};
obtaining for the test weld the values of (τ + Dₚ.tₚ)_{D} and (τ + Dₚ.t_{P})_{H} for the weld metal and for the heat affected zone where Dp is hydrogen diffusivity coefficient during the postweld heat treatment and tₚ is the holding time, and τ (cm²) is a hydrogen diffusion parameter in a welding operation under given conditions wherein
D, is a hydrogen diffusivity coefficient (cm²/sec.) in an arbitrary weld zone of each unit and tn is the time required for welding each unit layer;
determining for the test weld a value (Dₚ.tₚ) which corresponds to the larger of (D_{P}·tₚ)_{D} or (Dₚ·tₚ)_{H} by comparing those values, as a condition of the postweld heat treatment;
measuring for said multilayer weld the temperature at a suitable portion of the weld during the post weld heat treatment;
terminating the heat treatment of said multilayer weld at a time point when the time integrated value of the previously determined hydrogen diffusivity coefficient (Dₚᵢ) (cm²/sec.) at the measured temperature exceeds the previously determined value of (Dₚ.tₚ);
and wherein the critical hydrogen concentration, (Ccr), is related to the Vicker's hardness number, (Hv), such that (Ccr) ranges from 1.96 to 388 cc/100 g while (Hv) correspondingly ranges from 300 to 500.

In the accompanying drawings:
Figure 1 is a perspective view showing the conditions of test welding and a sampling position of a test piece;
Figure 2 is a diagrammatic view explanatory of the way to divide a welded joint into small elements for the analysis by the finite element method;
Figure 3 is a flow chart showing a programme for the analysis by the finite element method;
Figure 4 is a diagram showing the dependency on temperature of various thermal constants;
Figure 5 is a diagram showing the relation between the hydrogen diffusivity coefficient and the temperature;
Figure 6 is a schematic view explanatory of the restraint test specimen used in the cracking tests;
Figure 7 is a schematic perspective view showing the method for measuring diffusible hydrogen which is dissolved into weld metal by one pass of welding;
Fig. 8 is a diagram comparatively showing the actually measured and calculated values of the hydrogen concentration distribution at a time point when the final bead reaches an interpass temperature;
Fig. 9-(a) and (b) are the diagrams showing the relations between the hydrogen concentration immediately beneath the final pass of welds right after welding and the parameter (_{T}) of hydrogen diffusion at the time of welding for weld metal of steel weldments and for HAZ of A508 Class 3 weldments, respectively;
Fig. 10 is a schematic view of gas burners employed as auxiliary heating means for maintaining an interpass temperature at the time of welding;
Figs. 11 and 12 are diagrams showing the relation between welding conditions and the parameter (τ) of hydrogen diffusion with auxiliary heating for 21 4Cr―1 Mo steel weldments;
Fig. 13 is a diagram showing the same relation for A508 Class 3 weldments as Figs. 11 and 12.
Fig. 14-(a) is a diagram showing the influence of the hydrogen concentration distribution immediately after welding on the relation between the variation in hydrogen concentration in weld metal and treating conditions of the low temperature PWHT;
Fig. 14-(b) is the same diagram for HAZ as Fig. 14-(a);
Fig. 15-(a) is a diagram for weld metal showing the similar influence of the plate thickness;
Fig. 15-(b) is the similar diagram for HAZ as Fig. 15-(a);
Fig. 16-(a) is a diagram for weld metal showing the similar influence of the bevelling width;
Fig. 16-(b) is the similar diagram for HAZ as Fig. 16-(a);
Fig. 17 is a diagram showing the relation between the variations in the hydrogen concentration and PWHT conditions in a case where the bevelling width exceeds 36 mm;
Figs. 18-(a) and 18-(b) are the diagrams showing the results of cracking tests for 24Cr-1 Mo steel and A508 Class 3 material along with the distribution of hydrogen concentration, which were conducted for determining the crack-preventing critical hydrogen concentration;
Fig. 19 is a graph showing the relation between the crack-preventing critical hydrogen concentration in weld metal or in HAZ and maximum Vicker's hardness number of microstructure in the respective region;
Fig. 20 is a flow chart illustrating procedures for determining the conditions of the crack-preventing low temperature PWHT for various materials;
Fig. 21 is a schematic view showing PWHT in multilayer welding of a circumferential joint for a pressure vessel; and
Fig. 22 is a diagram showing the variations in the coefficient of hydrogen diffusion against time.

### PARTICULAR DESCRIPTION OF THE INVENTION

The method of the invention is hereafter described by way of fundamental tests conducted on 21 4Cr―1 Mo steel and A508 Class 3 material, results of the experiments and practical procedures for the respective steps.

### [Testing Method]

### 1. Test specimens and welding conditions

The base metal used in the tests was 200 mm thick rolled material of ASTM A387 and GR22 Class 2 and a forged A508 Class 3 material. Those chemical compositions and mechanical properties are shown in Table 1.

Table 2 below shows the submerged arc welding conditions.

The flux MF-29A or MF-27 was mainly used in the tests but the recently developed flux MF-29AX of low hydrogen level was used in certain cases.

Table 3 shows the chemical composition and mechanical properties of the weld metals.

### 2. Measurement of hydrogen concentration distribution in thick plate welds immediately after welding

Upon completion of welding, the distribution of hydrogen concentration in the direction of plate thickness immediately after the final bead cooled to an interpass temperature was measured, varying the preheating/interpass temperature and the plate thickness to clarify experimentally their influences on the distribution of hydrogen concentration in the weld metals. The obtained hydrogen distributions were used as comparative data against the calculated values to confirm the reliability of the program of finite element method for estimating the hydrogen distribution immediately after welding as described in the next paragraph. The shape and dimensions of the welding joint used for the measurement of diffusible hydrogen concentration are shown in Fig. 1 (1), while the sampling position of the test piece for its purpose is shown in Fig. 1 (2) in which the various lengths are in the unit of mm and indicated at 1 are trays for holding a cooling medium and dry ice and at 2 is a cut of the weld metal test piece.

### 3. Analysis of hydrogen diffusion during welding by finite element method

For handling the hydrogen diffusion during the welding operation, it is preconditional to reproduce the welding thermal cycle. However, our researches are directed to plates of a thickness of 50 mm or greater which require welding in a relatively large number of layers and the submerged arc welding process is generally utilized with high heat input, so that it is almost impossible to simulate on the test piece the welding thermal cycle which takes place when welding an actual structure. Therefore, the analysis based on the finite element method was utilized.

Fig. 2 illustrates an element division of a weld zone into small triangles of I-beveling welded with 2 passes per layer and having a penetration rate of 60%. In this figure, the reference numeral 6 denotes the weld of the first pass consisting of a weld portion 4 and a penetrated portion 5. Indicated at 6' is the weld of the 12th pass consisting of a weld portion 4' and a penetrated portion 5'. In this instance, the sum of residual hydrogen in the penetrated portion and a predetermined amount of hydrogen dissolved in the respective weld portion at the time of each weld is divided by the total weight of the weld and penetrated portions, allotting the mean value uniformly thereto as initial hydrogen concentration existing when welding each weld pass. The hydrogen concentration at the nodes on the surfaces were considered as being constantly held at zero throughout the analysis.

On the other hand, the calculation for the welding thermal history which is preconditional to the analysis of the hydrogen diffusion was performed with a heat input of 40 KJ/cm for 24Cr-1 Mo steel welds and 37 KJ/cm for A508 Class 3 welds and a heat efficiency of 65%, equivalently resdistributing them to the weld and penetrated portions.

Fig. 3 is a flow chart of a program used for the analysis. The time increment for each analysis was set in the range of 1 to 10 seconds to correspond with the cooling rate. The shift to the next pass was effected when a predetermined temperature was reached at a position located 10 mm inside the beveling face and 15 mm deep from the plate surface, compiling that temperature as an interpass temperature. With a larger plate thickness, the temperature was controlled by varying the measuring positions for a few times along the plate thickness in accordance with the progress of the welding operation. In the various tests using a test specimen as shown in Fig. 1, the welding thermal cycle was controlled by a CA thermocouple which was inserted at such measuring positions for conformity with conditions of calculation.

Figs. 4 and 5 show the dependency on temperature of the various thermal constants and the hydrogen diffusivity coefficient which were used in the calculations. With regard to the thermal transfer coefficient A, thermal conductivity B and specific heat C, the density was held constant in consideration of their dependency on temperature shown. For the dependency on temperature of the hydrogen diffusivity coefficient, the value indicated by solid lines in Fig. 5 was used.

### 4. Determination of hydrogen diffusivity coefficient of welded joints

The hydrogen diffusivity coefficient was determined by actually measuring the distributions of hydrogen concentration immediately after welding and after the low-temperature PWHT and comparing the measured values with calculated values as obtained under the same conditions.

### 5. Cracking test for determining critical hydrogen concentration free from transverse cracks

In order to know to which extent the concentration of residual hydrogen in the weld zone immediately after welding has to be reduced for the prevention of cracking, namely, in order to know the crack-free critical hydrogen concentration, cracking tests were conducted with the use of restrained test specimens as shown in Fig. 6, in which the respective dimensions are indicated in the unit of mm. The dimensions of h (plate thickness) X° (angle of beveling) and R (radius of curvature at the root of beveling) were varied in the cracking tests under the conditions shown in Table 4.

The low-temperature PWHT was performed in an annealing furnace. Leaving the test specimen at room temperature for two weeks after the low-temperature PWHT, vertical sections of the weld were cut out to check the existence of cracks by magnaflux detection and by naked eyes after etching.

Nextly, the hydrogen diffusion during PWHT was analyzed by the use of the thermal history which was obtained in the cracking test during the time interval from the completion of welding to the time point when the temperature of the test specimen cooled down to 100°C after the low temperature PWHT, thereby determining the hydrogen distribution in the weld zone at the temperature of 100°C. Thereafter, the crack-preventing critical hydrogen concentration was determined on the basis of the results of the cracking test and the corresponding distribution of hydrogen concentration.

### 6. Measurement of initial hydrogen content necessary for determining conditions of low temperature PWHT in accordance with the combination of base metal and welding materials

A test piece as shown in Fig. 7(1) (in which all the dimensions are indicated in the unit of mm) was welded with one pass in the arrowed direction which was, immediately after being quenched in a water bath with crushed ice, put in liquid nitrogen to fix hydrogen. Thereafter, four test pieces were cut off as shown in Fig. 7(2) for the determination of hydrogen. These test pieces were sealed in a vacuum container for about 20 days at room temperature and then subjected to determination of diffusible hydrogen by a vacuum extraction apparatus.

### [Test results and practical procedures]

### 1. Relation between hydrogen concentration immediately after welding and conditions of welding operation

Fig. 8 shows actually measured and calculated values of the hydrogen distribution in the weld metal of 2'-_{Q}Cr-1 Mo steel weldments when the final pass of the weld is cooled down to the interpass temperature. In this figure, the marks "0", "0" and "0" represent the actually measured values and the curves indicate the results of analysis. Both the actually measured and calculated values have peaks in the vicinity of a point immediately beneath the final layer, showing a higher value with a greater plate thickness. Generally, the calculated values coincide with the actually measured values indicatively of the reliability of the analyzing computer program. As mentioned hereinbefore, it is necessary to employ a large test specimen in order to simulate the cooling rate in actual welding involving a thick and wide plate. However, the hydrogen distribution in such a case can easily be obtained by the use of the analysing program.

Nextly, it is important to determine the relation between the hydrogen concentration immediately beneath the final bead and the conditions of welding operation for the prevention of transverse cracking induced in weld metal. With regard to the hydrogen concentration immediately beneath the newest bead after its pass of welding, it is determined by dissolved hydrogen from the arc column and residual hydrogen in the vicinity of the penetrated portion of the bead. It is easily conceivable that the latter is determined by dissolved hydrogen from the arc column during each pass of welding and residual hydrogen in the vicinity of the penetrated portion and the welding thermal history until that pass. In this instance, it is known that the dissolved hydrogen from the arc column in each pass welding is constant and according to the results of the study in the regard, the thermal history in each pass of welding is considered to be substantially the same. Therefore, the hydrogen concentration immediately beneath the penetrated portion after welding the final bead in multilayer welding can be determined from the mean hydrogen concentration in the weld immediately after welding the initial layer and one welding thermal history in the proximity of the final layer.

As to the hydrogen concentration in HAZ, the same consideration can be accepted because it becomes a function of hydrogen concentration in weld metal.

It is known from Fick's Second Law that a variation in hydrogen concentration during a small time period Ati at a certain point in proportional to Di-Ati where Di is the diffusivity coefficient at that point. It follows that the quantity of hydrogen which is diffusingly released from the weld zone in one welding thermal cycle is considered to be determined by which is obtained by dividing the thermal cycle into the small time periods Δti and adding Di·Δti corresponding to the respective Ati.

In view of the fact that the transverse cracking is most susceptible to occur in weld metal of 2 Cr―1 Mo steel weldment or in HAZ of A508 Class 3 weldments immediately beneath the final layer, the value of was determined on the basis of the thermal history of the final pass of welds, determining its relation with the hydrogen concentration in weld metal or in HAZ immediately beneath the penetrated portion of the final pass of welds. In Fig. 9-(a) for 2 Cr―1 Mo steel weldments, the abscissa represents τ for while the ordinate represents the hydrogen concentration in weld metal directly beneath the final bead immediately after welding the final pass, non-dimensionally in terms of the mean hydrogen concentration in the weld metal immediately after the initial welding. Here, the discussion is based on welding of one layer with one pass. In a case where one layer is welded with n-number of passes, this relation can be generalized by graduating the abscissa on the scale of (the same applies hereafter). The results of calculation shown in Fig. 9-(a) were obtained by varying the conditions of the welding operation over a wide range, including the thickness and width of plates and preheating and interpass temperatures. As clear from the figure, the relation between the hydrogen concentration in weld metal directly beneath the final pass immediately after welding and the parameter _{T} of hydrogen diffusion determined from the welding thermal history depending upon welding conditions can be expressed by a single curve. The same relation was obtained for HAZ of A508, Class 3 weldments as shown in Fig. 9-(b).

By the use of the diagram of Fig. 9-(a) or 9-(b), it becomes possible to dispense with the calculations which would otherwise be necessitated by variations in the mean hydrogen concentration Co,o in the weld immediately after welding the first layer, as a result of use of a flux of a different hydrogen level or a variation in the coefficient of hydrogen diffusion due to use of a different material. The hydrogen concentration directly beneath the final pass can be readily obtained as long as the value of Co,o or one welding thermal cycle in the vicinity of the final layer and the coefficient of hydrogen diffusion are known.

We now consider the relation between the parameter τ of hydrogen diffusion and the conditions of welding operations.

The foregoing description has dealt with the results where the next pass of welding is proceeded at a time point when the bead temperature reaches the level of the interpass temperature. However, in actual operation, there sometimes occurs a temperature drop during the pass interval which is elongated depending upon the size of a pressure vessel or the like. In such a case, the interpass temperature is maintained by an auxiliary heating means like gas burners as shown in Fig. 10. In this figure, indicated at 7 is a turning roller, at 8 a welding torch, at 9 a a gas burner and at 10 a shell course of a pressure vessel. While the welding bead temperature which has reached the interpass temperature is maintained at that level by the auxiliary heating means until the subsequent weld bead is deposited, it is now necessary to consider the influence of the auxiliary heating on the parameter _{T} of hydrogen diffusion.

With the auxiliary heating, the value of the parameter _{T} which is determined by one welding thermal cycle consists of the value of _{T} shown in Fig. 9 plus the contribution of the auxiliary heating, that is to say, the product D·Δta of the time interval Δta at which the welding of a next bead is deposited after the bead temperature reaching the interpass temperature and the coefficient D of hydrogen diffusion at the temperature. The value of Ata varies depending upon the welding conditions such as the interpass temperature, welding speed, dimensions of the base metal, for example, the diameter of a vessel when a girth welding to join the shell courses of a pressure vessel is performed.

Fig. 11 shows the relation between the pass interval and the parameter _{T} in a case where a joint of infinitely wide plate of Cr―1 Mo steel is welded at an interpass temperature of 200°C and, when the bead temperature reaches the interpass temperature at the time of welding each pass, it is maintained constantly at the interpass temperature by the auxiliary heating until the commencement of welding of the next pass. In this figure, the broken line indicates the relation between the time in which the bead temperature cools off to the interpass temperature after the welding of the bead and the value of _{T} as determined by the welding thermal cycle at that time, namely, the value of of Fig. 9-(a). In this instance, the preheating zones on opposite sides of the weld were locally preheated to 200°C over a width corresponding to the plate thickness of 50 mm or 100 mm. The value of _{T} thus obtained was 0.041 cm² with a plate thickness of 50 mm and 0.022 cm² with a plate thickness of 100 mm. The value of _{T} resulting from overall preheating was 0.041 cm² with a plate thickness of 50 mm and 0.023 cm² with a plate thickness of 100 mm, which were substantially the same as the values in the case of local preheating. It is known therefrom that, in the multilayer welding for plates of extremely great thickness, the preheating in the initial stage imposes almost no influence on the welding thermal cycle of the final layer due to dissipation of heat over a long time period before completion of the welding. Therefore, the relation between the cooling time to the interpass temperature after the final pass of welding and for a plate thickness of 250 mm was determined on the welding of the final ten passes alone without preheating.

In Fig. 11, the straight line which extends out of the broken line indicates the relation between the time Ata in which the welding of the next pass is initiated after the bead temperature reaching the interpass temperature and the increase in τ due to the auxiliary heating, namely, the relation of D·Δta. Therefore, the gradient of the straight line equals the coefficient of hydrogen diffusivity at the interpass temperature. It is clear therefrom that the pass interval imposes a great influence on the parameter _{T} in consideration of the auxiliary heating. Fig. 12 shows their relation in both cases where the interpass temperature is 150°C and 250°C. Upon comparing this figure with Fig. 11, it is observed that the influence of the auxiliary heating on the parameter _{T} becomes greater with a higher interpass temperature although its effect is unexpectable at the temperature of 150°C.

Thus, the hydrogen concentration in weld metal of 2 Cr―1Mo steel weldments immediately after welding under given conditions can readily be obtained from the diagram of Fig. 9-(a) by equivalently substituting thereinto the value of τ as determined by Fig. 11 or Fig. 12.

As for the hydrogen concentration in HAZ of A508 Class 3 weldments, relationship shown in Fig. 13 was obtained. So, its value immediately after welding can be obtained by combining Fig. 9-(b) and Fig. 13.

### 2. Relation between variations in hydrogen concentration during low temperature PWHT and treating conditions

### 2-1 Influence of initial hydrogen distribution

Since the transverse weld cracking is most susceptible to occur in the vicinity of the peak of the hydrogen concentration, it is important to clarify the relation between the variations in the peak values of the hydrogen concentration both in weld metal and in HAZ during the low temperature PWHT and the treating conditions in order to prevent the transverse cracking. This paragraph deals with the influence of the hydrogen concentration distribution immediately after welding on that relation.

Fig. 14-(a) illustrates the relation between the peak value of the hydrogen concentration in weld metal during the low temperature PWHT (LTPWHT) and the treating conditions. In the diagram of Fig. 14-(a), the ordinate represents the ratio of the peak value C of the hydrogen concentration in the low temperature PWHT in weld metal to the hydrogen concentration Co immediately beneath the final bead after welding, while the abscissa represents the sum of the value of the parameter _{T} of hydrogen diffusion during welding and the product Dp-tp of the coefficient of hydrogen diffusivity at the temperature of the PWHT and the holding time. Thus, the diagram of Fig. 14-(a) shows, by way of the relation between C/Co and (τ + Dₚ·tₚ), the influence of the initial hydrogen distribution on the relation between the variation in the peak value of the hydrogen concentration in the low temperature PWHT and the treating conditions, namely, the influence of the hydrogen distribution immediately after the bead temperature reaching the level of the interpass temperature upon completion of welding. The initial hydrogen concentration distribution was varied by changing the preheating and interpass temperatures in various ways. It is observed therefrom that, even if the initial hydrogen distribution is varied, it is possible to express the relation between the variations in the peak value of the hydrogen concentration and the treating conditions substantially by a single curve based on the relation of C/Co and (τ + Dp·tp).

The similar relation was obtained for HAZ as shown in Fig. 14-(b). The change of hydrogen concentration in HAZ through PWHT except for the early stage of it can also be expressed by a single curve regardless of hydrogen concentration distribution immediately after welding.

### 2-2 Influences of plate thickness

The diagram of Fig. 15-(a) shows the influence of the plate thickness on the relation between the peak values in weld metals and the treating conditions. As clear therefrom, no influence of the plate thickness is observed in the initial stage of the low temperature PWHT. This is because the peak value of the hydrogen concentration is located immediately beneath the final bead and the hydrogen diffusion at that position is greatly influenced by the plate surface. Further, as the heat treatment proceeds, the influence of the plate thickness is gradually manifested due to inward shift of the peak position of the hydrogen concentration. Judging from the conditions of low temperature PWHT which prevent the cracking, the value of (τ + Dₚ·tₚ) should be smaller than 1.5 cm² at largest in the case of 2 Cr―1 Mo steel weldments by submerged arc welding process with the heat input of 40 KJ/cm. Therefore, with a plate thickness in excess of 100 mm, the preventing condition for a cold cracking induced in weld metal of 2'Cr-1 Mo steel weldments can be obtained from the relation between C/Co and (_{T} + Dp-tp) for the plate thickness of 100 mm.

The similar relation for HAZ was obtained as indicated in Fig. 15-(b).

### 2-3 Influence of beveling width

Fig. 16-(a) shows the influence of the beveling width of the weld on the relation between C/Co in weld metal and (τ + D_{P}·tₚ). Fig. 16-(b) is for HAZ. It is clear therefrom that the change of the hydrogen concentration is delayed with a larger beveling width since the gradient of hydrogen concentration in a direction perpendicular to the weld line becomes smaller as the beveling width is increased. When considering the hydrogen diffusion in the weld, it is often discussed as a one-dimensional diffusion in the direction of plate thickness, ignoring the diffusion from the weld to the base metal. However, in view of Figs. 15 and 16 which show the influence of the beveling width rather than that of the plate thickness, such a discussion is obviously meaningless. Although Fig. 16-(a) shows the influence of the beveling width of up to 36 mm, it is the general practice in the welding in flat position to design the beveling in a constant width taking into account the transverse contraction of the weld, for ensuring a high welding efficiency. Therefore, the beveling width for plates of a thickness of about 300 mm may be taken as about 36 mm at maximum. On the other hand, in horizontal position, the beveling width is increased with a greater plate thickness and may exceed 36 mm in some cases. Therefore, nextly considered is the relation between C/Co in weld metal and (τ + Dₚ·tₚ) in a case where the beveling width is greater than 36 mm.

With a heavier plate thickness, the diffusion takes place in a greater degree in the direction of plate width than in the direction of plate thickness. Now, assuming that the diffusion occurs only in the direction of plate width according to Fick's Second Law, the ratio of the hydrogen concentration C at the center of the weld during the low temperature PWHT to the initial hydrogen concentration Co can be expressed simply as C/Co=Φ (W/4√τ + Dₚ·tₚ), in which Φ is an error function. The influence of a beveling width greater than 36 mm can thus be approximately expressed by arranging the results of the case of h = 150 mm and W = 36 mm of Fig. 16-(a) into the relation between C/Co and .

The solid line in Fig. 17 is a plot of the thus obtained relation between the variation in the hydrogen concentration in the low temperature PWHT, treating conditions and beveling width. However, this relation fails to sufficiently take into account the diffusion in the direction of plate thickness except for the case where W = 36 mm, underestimating the diffusion in an increasing degree as the beveling width becomes larger than 36 mm. As a result, C/Co is given a value which is greater than its actual value. However, as mentioned hereinbefore, the diffusion in the direction of plate thickness is considered to take place in a small degree as compared with that in the direction of plate width in a case where the plate thickness is sufficiently large relative to the beveling width, approximately establishing the relation shown. Therefore, the relation of C/Co and (τ + Dₚ·tₚ ) in the case where h = 150 mm and W = 30 mm of Fig. 16 was arranged into the relation of C/Co and as indicated by a curve of broken line in Fig. 17. Upon comparing the curves of solid and broken lines, it will be clear that the relation between C/Co and undergoes almost no changes in spite of variations in W. Thus, it is possible to obtain safe and approximately correct conditions for the low temperature PWHT for weld metal by applying the curve of solid line to beveling widths greater than 36 mm.

The same relation with regard to the change of hydrogen concentration in HAZ where a beveling width is greater than 37 mm, can easily be obtained by making use of the relation in case of plate thickness and beveling width being 150 mm and 37 mm, which is shown in Fig. 16-(b).

### 3. Critical hydrogen concentration for preventing transverse cracking in weld zone in butt welding

Fig. 18-(a) shows the results of cracking tests under different conditions of welding and low temperature PWHT along with hydrogen distributions in the respective test conditions. Since prevention of the cold cracking is considered to depend on the cooling rate to the level of 100°C, the critical hydrogen concentration for the prevention of cracking is expressed by values at the time when the test pieces are cooled to 100°C. The curves in this figure indicate the hydrogen concentration distributions in the cooled test pieces at 100°C, of which curves of broken lines are of test pieces with a crack and the curves of solid lines are of test pieces without a crack. It will be clear therefrom that the crack-preventing critical hydrogen concentration in the weld in butt welding of 21 4Cr―1 Mo steel is about 3.3 cc/100 gr at a peak value.

On the other hand, as for A508 Cl.3 weldments, its susceptibility to the transverse weld cracking induced in HAZ depends upon the extent of the segregation of alloying elements and impure elements, such as C, Mn, Si, Mo, S, and so forth. In other words, the critical hydrogen concentration changes depending upon whether HAZ contains a so-called inverse V segregation zone, or not, as shown in Fig. 18-(b). This is because such a segregation hardens the microstructure of HAZ to a high degree.

From these data, we can introduce a relation practically useful to determine the critical hydrogen concentration under which any transverse weld cracking will not occur either in weld metal or in HAZ. Fig. 19 shows the relation between the hydrogen concentration and the microstructure in weld zone in terms of maximum Vicker's hardness number with regard to the occurrence of the crack. So, a straight line in the figure shows the relation between the critical hydrogen concentration (Ccr) and maximum Vicker's hardness number in weld zone (Hv), as is represented by an equation: where (Hv) is in the range of 300 to 500. Inserting the limiting values of (Hv) (300 and 500) in equation (1) we get a corresponding range of values of (Ccr) of 1.96 to 3.88 cc/100 g.

Using this relationship, we can easily determine the critical hydrogen concentration depending upon the base metal and welding conditions, such as welding materials, weld heat input, and so forth through the maximum Vicker's hardness number in weld zone produced under the respective conditions.

As a result, using the value of (Ccr) obtained from the above equation, we can determine the minimum condition of low-temperature PWHT required to prevent the transverse crack induced in multi-layer welds. Of course, in order to determine the practical condition of PWHT, the value of (Ccr) should be estimated lower to a certain extent than the value obtained from the equation because the factor of safety should be modified depending upon the importance of the structure, accuracy of nondestructive inspection employed for weld zone, and so forth.

### 4. Condition for preventing cracking through low temperature PWHT

As mentioned hereinbefore, the conditions for preventing cracking through low temperature PWHT depend on factors such as the shape and dimensions of the weld, the hydrogen level of the flux, sort of the base metal or its combination with welding materials and the conditions of the welding operation. As an example the conditions for a particular operation for 2-!Cr-1 Mo steel weldments are determined by the following procedures.
(1) For given plate thickness at the weld, preheating and interpass temperatures, number of weld passes per layer, and pass intervals, decide the parameter which governs the hydrogen diffusion at the time of welding by the use of the diagram of Fig. 11 or Fig. 12.
(2) Find in Fig. 9-(a) the value of the hydrogen concentration Co which is determined by the parameter. Here, Co,o represents the mean hydrogen concentration in the weld immediately after welding the first pass and is 4.74 cc/100 g in the case of submerged arc welding using the flux MF-29A.
(3) Obtain the values of the crack-preventing critical hydrogen concentration Ccr from the relation between Ccr and maximum Vicker's hardness number in weld metal, mentioned in the preceding paragraph and its ratio Ccr/Co to the hydrogen concentration Co immediately after welding.
(4) Plot the values of Ccr/Co of the preceding step (3) on the ordinate of the diagram of Fig. 16-(a) or Fig. 17, reading out the necessary treating conditions (_{T} + Dp-tp) on the abscissa according to the given plate thickness and v beveling width.
(5) Subtract the value of τ of the step (1) from the value of (_{T} + Dp.tp) of the step (4) to obtain the low temperature PWHT conditions Dp-tp suitable for the plate thickness, preheating and interpass temperatures, number of weld passes per layer, pass intervals, maximum Vicker's hardness number in weld zone, and beveling width as specified in the steps (1) through (4). Here, the values of Dp and tp represent the hydrogen diffusivity coefficient and the holding time at the treating temperature, respectively, so that the holding time for a given treating temperature can be obtained according to the relation between the hydrogen diffusivity coefficient and the temperature. The same condition of PWHT required to prevent the occurrence of a cold cracking in other low alloy steel weldments can be evaluated by following the procedure presented in Fig. 20.

Fig. 21 schematically shows the PWHT in multi-layer welding of a circumferential joint of a pressure vessel, wherein a shell course of a vessel 1 which is rotated on turning rollers 7 in the arrowed direction is heated at two positions by burners 9A and 9B while measuring the temperature of the shell course 1 at six different positions T, to T₆. There are no restrictions on the numbers of the burners and measuring points or on the measuring positions or method. However, it is preferred to provide the burners and measuring points as many positions as possible in order to enhance the accuracy of the heat control. The dissipation of diffusible hydrogen is improved all the more in a case where the shell course is heated on both the inner and outer sides thereof.

The diagram of Fig. 22 shows the relation between the lapse of time in the course of measurement at the respective measuring points of the temperatures of the shell course 1 heated by burners 9A and 9B and the hydrogen diffusivity coefficient (Dₚᵢ) at the respective temperatures. In order to assist understanding, the diagram shows the positions of the burners 9A and 9B relative to the measuring points. It will be seen therefrom that the hydrogen diffusivity coefficient (Dₚᵢ) has a pattern of declining from T, to T₃ and from T₄ to T₆.

While rotating the vessel for the LTPWHT in the above-described manner, the value of Dp, which varies with lapses of time is time-integrated until its cumulative value reaches Dₚ·tₚ determined in the step (5). Upon detection of the time point when the time integration of Dₚᵢ reaches Dₚ·tₚ, the LTPWHT is terminated since the concentration of diffusible hydrogen at the peak position is smaller than the critical hydrogen concentration Ccr at that time point.

In a welding operation other than the circumferential welding of a vessel, for instance, in an operation for a seam welding or for welding a nozzle to a pressure vessel, the weld line is uniformly heated along the entire length thereof so that the temperatures measured only at one arbitrary point may be used for the control of the PWHT.

It will be appreciated from the foregoing description that, according to the method of the present invention, it becomes possible to judge the terminating point of the LTPWHT correctly and to improve the quality control by precluding the cracking due to insufficient LTPWHT or uneconomical excessive PWHT, so called intermediate stress relief annealing.

## Claims

1. A method for the low-temperature PWHT in multilayer welding, comprising the steps of: determining the residual hydrogen concentration Co (cc/100 g) directly beneath the final welded layer immediately after completion of welding;
determining a crack-preventing critical hydrogen concentration Ccr (cc/100 g) to obtain a ratio of Ccr/Co;
determining the value of a product D_{P}·t_{P} of a hydrogen diffusivity coefficient Dₚ(cm²/sec.) during the heat treatment and a holding time tp(sec.) where a currently reached hydrogen concentration C (cc/100 g) become equal to the critical hydrogen concentration Ccr, on the basis of the relation of a ratio C/Co of the current hydrogen concentration C(cc/100 g) to the residual hydrogen concentration Co and a sum of a parameter τ (cm²) of hydrogen diffusion of the formula given below and the product of ^{D}p^{·t}p^{;}
measuring the temperature of the heat treatment at a suitable position of the weld;
terminating the heat treatment at a time point when a time-integrated value of a hydrogen diffusivity coefficient Dₚᵢ(cm²/sec.) at the measured temperature exceeds the value of Dₚ·tₚ under given conditions wherein,
PWHT: postweld heat treatment,
Dᵢ: a hydrogen diffusivity coefficient (cm²/sec.) in an arbitrary weld portion during welding each unit layer; and
tn: time (sec.) required for welding each unit layer.
and wherein the critical hydrogen concentration, (Ccr) is related to the Vicker's hardness number, (Hv) such that (Ccr) ranges from 1.96 to 3.88 cc/100 g while (Hv) correspondingly ranges from 300 to 500.

2. A method for the low-temperature PWHT as set forth in claim 1, comprising determining the parameter _{T} of hydrogen diffusion and the dissolved hydrogen concentration Co,o (cc/100 g) under given welding conditions, and determining Co on the basis of the relation between the parameter τ and Co/Co,o.

3. A method for the low-temperature PWHT as set forth in claim 1 or 2, comprising heating a circumferential weld of a rotated heavily thick vessel by more than one burner, measuring the temperature of said weld at an arbitrary point thereof to obtain variations in a hydrogen diffusivity coefficient Dpi against time, and detecting the time point when the time integrated value of said coefficient Dpi exceeds the value of Dp.tp.

4. A method for the low temperature PWHT as set forth in claim 1 or 2, comprising heating a butt weld line from one side thereof by a plural number of fixed burners while measuring temperatures at arbitrary different points on the other side of said weld line to obtain variation in the hydrogen diffusivity coefficient Dₚᵢ against time, and detecting a time point when the time integrated value of Dₚᵢ exceeds the value of Dₚ·tₚ.

5. A method for the low temperature postweld heat treatment in multilayer welding, comprises the steps of:
obtaining the residual hydrogen concentration (Co)e and (C_{O})_{H} (cc/100 g) directly beneath the finally welded layer immediately after completion of multilayer welding, where (Co)_{D} and (Co)_{H} are for weld metal (deposited metal) and for heat affected zone, respectively;
obtaining the critical hydrogen concentration for prevention of cracking (Ccr)_{D} and (Ccr)_{H} for the weld metal and for the heat affected zone, respectively, which depend upon the maximum residual stress and maximum Vicker's hardness number of microstructure in weld zone;
obtaining the values of (Ccr/Co)_{D} and (Ccr/Co)_{H}, ratio of the critical hydrogen concentration (Ccr)ₑ and (Ccr)_{H} for prevention of cracking both in the weld metal and the heat affected zone to the residual hydrogen concentration (Co)_{D} and (Co)_{H};
obtaining the values of (C/Co)_{D} and (C/Co)_{H} for the weld metal and for the heat affected zone, the ratio of the hydrogen concentration in the weld zone (C)_{D} and (C)_{H} which are lessened by the low temperature postweld heat treatment to the residual hydrogen concentration (Co)_{D} and (Co)_{H};
obtaining the values of (τ + D_{P}·tₚ)_{D} and (τ + Dₚ·tₚ)_{H} for the weld metal and for the heat affected zone where Dp is hydrogen diffusivity coefficient during the postweld heat treatment and tp is the holding time, and τ (cm²) is a hydrogen diffusion parameter in a welding operation under given conditions wherein
D, is a hydrogen diffusivity coefficient (cm²/sec.) in an arbitrary weld zone of each unit and tn is the time required for welding each unit layer;
determining a larger value (Dₚ·tₚ) of (Dₚ·tₚ)_{D} or (Dₚ·tₚ)_{H} by comparing those values, as a condition of the postweld heat treatment;
measuring the temperature at a suitable portion of the weld during the postweld heat treatment, terminate the heat treatment at a time point when the time integrated value of the hydrogen diffusivity coefficient (Dₚᵢ) (cm²/sec.) at the measured temperature exceeds the value of (Dₚ·tₚ),
and wherein the critical hydrogen concentrations (Ccr)_{D} and (Ccr)_{H} are related to the Vicker's hardness numbers, (Hv)_{D} and (Hv)_{H} respectively such that (Ccr)_{D} and (Ccr)_{H} range from 1.96 to 3.88 cc/100 g while (Hv)_{D} and (Hv)_{H} correspondingly range from 300 to 500.

6. A method for the low temperature PWHT of a multi-layer weld characterised by the steps of: determining for a test weld similar to said multilayer weld the residual hydrogen concentration Co (cc/100 g) directly beneath the final welded layer immediately after completion of welding;
determining for the test weld a crack-preventing critical hydrogen concentration Ccr (cc/100 g) to obtain a ratio of Ccr/Co;
determining for the test weld a value of a product Dp.tp of a hydrogen diffusivity coefficient Dp(cm²/sec.) during the heat treatment and a holding time tp(sec.) where a currently reached hydrogen concentration C (cc/100 g) becomes equal to the critical hydrogen concentration Ccr, on the basis of the relation of a ratio C/Co of the current hydrogen concentration C (cc/100 g) to the residual hydrogen concentration Co and a sum of a parameter _{T} (cm²) of hydrogen diffusion of the formula given below and the product of D_{P}·tₚ;
measuring for said multilayer weld the temperature of the heat treatment at a suitable position of the weld;
terminating the heat treatment of said multilayer weld at a time point when a time integrated value of the previously determined hydrogen diffusivity coefficient Dₚᵢ(cm²/sec.) at the measured temperature exceeds the previously determined value of Dₚ·tₚ. wherein,
PWHT: postweld heat treatment,
Dᵢ: a hydrogen diffusivity coefficient (cm²/sec.) in an arbitrary weld portion during welding each unit layer; and
tn: time (sec.) required for welding each unit layer,
and wherein the critical hydrogen concentration, (Ccr), is related to the Vicker's hardness number, (Hv), such that (Ccr) ranges from 1.96 to 3.88 cc/100 g while (Hv) correspondingly ranges from 300 to 500.

7. A method for the low temperature postweld heat treatment of a multilayer weld, characterised by the steps of;
obtaining for a test weld similar to said multilayer weld, the residual hydrogen concentration (Co)_{D} and (Co)_{H} (cc/100 g) directly beneath the finally welded layer immediately after completion of multilayer welding, where (Co)_{D} and (Co)_{H} are for weld metal (deposited metal) and for heat affected zone, respectively;
obtaining for the test weld the critical hydrogen concentration for prevention of cracking (Ccr)_{D} and (Ccr)_{H} for the weld metal and for the heat affected zone, respectively, which depend upon the maximum residual stress and maximum Vicker's hardness number of the microstructure in the weld zone;
obtaining for the test weld the values of (Ccr/Co)_{D} and (Ccr/Co)_{H}, the ratio of the critical hydrogen concentration (Ccr)_{D} and (Ccr)_{H} for prevention of cracking both in the weld metal and the heat affected zone to the residual hydrogen concentration (Co)_{D} and (Co)_{H};
obtaining for the test weld the values of (C/Co)_{D} and (C/Co)_{H} for the weld metal and for the heat affected zone, the ratio of the hydrogen concentration in the weld zone and the heat affected zone (C)_{D} and (C)_{H} which are lessened by the low temperature postweld heat treatment to the residual hydrogen concentration (Co)_{D} and (Co)_{H};
obtaining for the test weld the values of (τ + Dₚ·tₚ)_{D} and (τ + Dₚ·tₚ)_{H} for the weld metal and for the heat affected zone where Dp is hydrogen diffusivity coefficient during the postweld heat treatment and tₚ is the holding time, and τ (cm²) is a hydrogen diffusion parameter in a welding operation under given conditions wnerein
D, is a hydrogen diffusivity coefficient (cm²/sec.) in an arbitrary weld zone of each unit and tn is the time requird for welding each unit layer;
determining for the test weld a value (Dₚ·tₚ) which corresponds to the larger of (Dₚt_{P})_{D} or (D_{P}·t_{P})_{H} by comparing those values, as a condition of the postweld heat treatment;
measuring for said multilayer weld the temperature at a suitable portion of the weld during the postweld heat treatment,
terminating the heat treatment of said multilayer weld at a time point when the time integrated value of the previously determined hydrogen diffusivity coefficient (Dₚᵢ) (cm²/sec.) at the measured temperature exceeds the previously determined value of (Dₚ·tₚ), and
wherein the critical hydrogen concentrations (Ccr)_{D} and (Ccr)_{H} are related to the Vicker's hardness numbers, (Hv)_{D} and (Hv)_{H} respectively such that (Ccr)_{D} and (Ccr)_{H} range from 1.96 to 3.88 cc/100 g while (Hv)_{D} and (Hv)_{H} correspondingly range from 300 to 500.

## Revendications

1. Un procédé de traitement thermique de joints soudés par soudure à multicouches, comportant les étapes de:
déterminer la concentration d'hydrogène résiduel Co (cm³/100g) directement au-dessus de la couche finale soudée immédiatement après la fin du soudage;
déterminer une concentration d'hydrogène critique évitant les criques Ccr (cm³/100 g) pour obtenir un rapport de Ccr/Co;
déterminer la valeur d'un produit Dp.tp d'un coefficient de diffusion d'hydrogène Dp (cm²/sec) pendant le traitement thermique et un temps de maintien tp (sec) où une concentration en hydrogène couramment atteinte C (cm³/100 g) devient égale à la consommation critique en hydrogène Ccr, sur la base de la relation d'un rapport C/co de la concentration courante en hydrogène C (cm³/100 g) à une concentration en hydrogène résiduel Co et une somme d'un paramètre τ (cm²) de la diffusion d'hydrogène de la formule donnée ci-dessous et le produit de Dₚ·tₚ;
mesurer la température du traitement thermique en une position appropriée de la soudure;
terminer le traitement thermique à un moment donné lorsqu'une valeur intégrée de temps du coefficient de diffusion d'hydrogène Dₚᵢ (cm²/sec) à la température mesurée est supérieure à la valeur de Dₚ·tₚ dans les conditions données dans laquelle:
Dᵢ: un coefficient de diffusion d'hydrogène (cm²/sec) dans une zone de soudure arbitraire pendant le soudage de chaque couche unitaire; et
tn: temps (sec) nécessaire pour souder chaque couche unitaire, et dans laquelle la concentration critique en hydrogène (Ccr) est rapportée à l'indice de dureté Vicker (Hv) de sorte que (Ccr) se situe entre 1,96 et 3,88 cm³/100 g tandis que (Hv) se situe de façon correspondante entre 300 et 500.

2. Un procédé pour le traitement thermique de joints soudés à basse température comme spécifié dans la revendication 1, consistant à déterminer le paramètre τ de la diffusion d'hydrogène et la concentration d'hydrogène dissous en Co,o (cm³.100 g) sous les conditions données de soudage, et à déterminer Co sur la base de la relation entre le paramètre τ et Co/Co,o.

3. Un procédé pour le traitement thermique de joints soudés à basse température comme spécifié dans la revendication 1 ou 2, consistant à chauffer une soudure circonférentielle d'un récipient rotatif fortement épais par plus d'un brûleur; à mesurer la température de ladite soudure en un point arbitraire de cette dernière pour obtenir des variations dans un coefficient de diffusion d'hydrogène Dₚᵢ en fonction du temps, et à détecter le moment donné où la valeur intégrée de temps dudit coefficient Dₚᵢ est supérieure à la valeur de Dp.tp.

4. Un procédé pour le traitement thermique de joints soudés à basse température comme spécifié dans la revendication 1 ou 2, consistant à chauffer une ligne de soudure de joints d'un côté de cette dernière par une pluralité de brûleurs fixes tout en mesurant les températures à différents points arbitraires de l'autre côté de ladite ligne de soudure pour obtenir une variation dans le coefficient de diffusion d'hydrogène Dₚᵢ par rapport au temps, et à détecter à un moment donné lorsque la valeur intégrée de temps de Dₚᵢ est supérieure à la valeur de Dₚ·t_{P}.

5. Un procédé pour le traitement thermique de joints soudés à basse température en soudure à multicouches, est constitué des étapes de:
obtenir la concentration en hydrogène résiduel (Co)_{D} et (Co)_{H} (cm³/100 g) directement au-dessus de la couche finalement soudée, immédiatement après la fin de la soudure multicouche, où (Co)_{D} et (C_{O})_{H} sont pour le métal soudé (métal déposé) et pour la zone soumise à la chaleur, respectivement;
obtenir la concentration critique en hydrogène pour éviter la formation de criques (Ccr)_{D} et (Ccr)_{H} pour le métal soudé et pour la zone soumise à la chaleur, respectivement, qui dépend de la contrainte résiduelle maximale et de indice dureté Vicker maximale de la microstructure dans la zone soudée;
obtenir les valeurs de (Ccr/Co)_{D} et (Ccr/Co)_{H}, par rapport de la concentration critique en hydrogène (Ccr)_{D} et (Ccr)_{H} pour éviter la formation de criques à la fois dans le métal soudé et dans la zone soumise à la chaleur à la concentration en hydrogène résiduel (Co)_{D} et (Co)_{H};
obtenir les valeurs de (C/Co)_{D} et (C/Co)_{H} pour le métal soudé et pour la zone soumise à la chaleur, le rapport de la concentration en hydrogène dans la zone soudée (C)_{D} et (C)_{H} qui sont réduits par le traitement thermique des joints soudés à basse température, à la concentration en hydrogène résiduel (Co)_{D} et (Co)_{H};
obtenir les valeurs de (τ + Dₚ·tₚ)_{D} et (τ + Dₚ·tₚ)_{H} pour le métal soudé et pour la zone soumise à la chaleur où Dp est le coefficient de diffusion de l'hydrogène pendant le traitement thermique des joints soudés et tp est le temps de maintien, et τ (cm²) est un paramètre de diffusion de l'hydrogène dans une technique de soudure sous les conditions données où Dᵢ est un coefficient de diffusion de l'hydrogène (cm²/sec) dans une zone de soudure arbitraire de chaque unité et tn est le temps nécessaire pour souder chaque couche unitaire;
déterminer une valeur plus importante (Dₚ·tₚ) de (Dₚ·tₚ)_{D} ou (Dₚ·tₚ)_{H} en comparant ces valeurs, comme une condition du traitement thermique des joints soudés;
mesurer la température en une zone appropriée de la soudure pendant le traitement thermique des joints soudés,
terminer le traitement thermique à un moment donné lorsque la valeur intégrée de temps du coefficient de diffusion d'hydrogène (Dₚᵢ) (cm²/sec.) à la température mesurée est supérieure à la valeur de (Dₚ·tₚ), et dans lequel les concentrations critiques en hydrogène (Ccr)_{D} et (Ccr)_{H} sont en rapport avec les indices de dureté Vickers, (Hv)_{D} et (Hv)_{H} respectivement de sorte que (Ccr)_{D} et (Ccr)_{H} se situent entre 1,96 et 3,88 cm³/100 g tandis (Hv)_{D} et (Hv)_{H} se situent de façon correspondante entre 300 et 500.

6. Un procédé pour le traitement thermique de joints soudés à basse température d'une soudure multi-couches, caractérisé par les étapes de:
déterminer pour une soudure d'essai ouverte à ladite soudure multi-couches, la concentration en hydrogène résiduel Co (cm³/100 g) est directement au-dessus de la couche soudée finale immédiatement après la fin du soudage;
déterminer pour la soudure d'essai une concentration critique en hydrogène évitant les criques Ccr (cm³/100 g) pour obtenir un rapport de Ccr/Co;
déterminer pour la soudure d'essai la valeur d'un produit Dp.tp d'un coefficient de diffusion d'hydrogène Dp (cm²/sec) pendant le traitement thermique et un temps de maintien tp (sec) ou une concentration d'hydrogène couramment atteinte C (cc/100 g) devient égale à la concentration critique en hydrogène Ccr, sur la base de la relation d'un rapport C/Co de la concentration courante en hydrogène C (cm³/100 g) à la concentration d'hydrogène résiduel Co et une somme d'un paramètre _{T} (cm²) de diffusion en hydrogène de la formule donnée ci-dessous et le produit de Dp.tp;
mesurer pour cette soudure multicouches, la température du traitement thermique en une position donnée de la soudure;
terminer le traitement thermique de cette soudure multi-couches à un moment donné lorsqu'une valeur intégrée de temps du coefficient de diffusion d'hydrogène déterminée au préalable Dₚᵢ (cm²/sec) à la température mesurée dépasse la valeur déterminée au préalable de D_{P}·tₚ. où
Dᵢ: un coefficient de diffusion d'hydrogène (cm²/sec.) dans une zone de soudure arbitraire pendant le soudage de chaque couche unitaire; et
tn: temps (sec) nécessaire pour souder chaque couche unitaire et dans lequel la concentration en hydrogène est critique (Ccr), est en rapport avec l'indice de dureté Vicker, (Hv), de sorte que (Ccr) se situe entre 1,96 et 3,88 cm³/100 g tandis (Hv) se situe de façon correspondante entre 300 et 500.

7. Un procédé pour le traitement thermique de joints soudés à basse température, d'une soudure multicouches, caractérisé par les étapes de:
obtenir pour une soudure d'essais similaires à cette soudure multicouches, la concentration d'hydrogène résiduel (Co)_{D} et (Co)_{H} (cm³/100 g) directement au-dessus de la couche finalement soudée, immédiatement après la fin du soudage multicouches, où (Co)_{D} et (Co)_{H} sont pour le métal soudé (métal déposé) et pour la zone soumise à la chaleur, respectivement;
obtenir pour la soudure d'essais la concentration critique en hydrogène pour éviter la formation de criques (Ccr)_{D} et (Ccr)_{H} pour le métal soudé et pour la zone soumise à la chaleur, respectivement, qui dépend de la contrainte résiduelle maximale et de l'indice de dureté Vicker de la microstructure dans la zone de soudage;
obtenir pour la soudure d'essais les valeurs de (Ccr/Co)_{D} et (Ccr/Co)_{H}, le rapport de la concentration d'hydrogène critique (Ccr)_{D} et (Ccr)_{H} pour éviter la formation de criques à la fois dans le métal soudé et la zone soumise à la chaleur à la concentration d'hydrogène résiduel (Co)_{D} et (Co)_{H};
obtenir pour la soudure d'essais les valeurs de (C/Co)ₒ et (C/Co)_{H} pour le métal soudé et pour la zone soumise à la chaleur, le rapport de la concentration d'hydrogène dans la zone soudée et la zone soumise à la chaleur (C)_{D} et (C)_{H} qui sont réduites par le traitement thermique de joints soudés à basse température à la concentration d'hydrogène résiduel (Co)_{D} et (Co)_{H};
obtenir pour la soudure d'essais les valeurs de (τ + Dₚ·tₚ)_{D} et (τ + Dₚ·tₚ)_{H} pour le métal soudé et pour la zone soumise à la chaleur, où Dp est le coefficient de diffusion d'hydrogène pendant le traitement thermique de joints soudés et tp est le temps de maintien, et τ (cm²) est un paramètre de diffusion hydrogène dans une opération de soudage sous les conditions données où Dᵢ est un coefficient de diffusion d'hydrogène (cm²/sec) dans une zone soudée arbitraire de chaque unité et tn est le temps nécessaire pour souder chaque couche unitaire;
déterminer pour la soudure d'essais à une valeur (Dₚ·tₚ) qui correspond à la plus grande valeur de (Dₚ·tₚ)_{D} ou (Dₚ·tₚ)_{H} en comparant ces valeurs, comme une condition du traitement thermique des joints soudés;
mesurer pour cette soudure multicouches la température en une zone appropriée de la soudure pendant le traitement thermique des joints soudés;
terminer le traitement thermique de cette soudure multi-couches à un moment donné lorsque la valeur intégrée de temps du coefficient de diffusion d'hydrogène déterminé au préalable (Dₚᵢ) (cm²/sec), à la température mesurée surpasse la valeur déterminée au préalable (Dp.tp), et
dans lequel les concentrations critiques d'hydrogène (Ccr)_{D} et (Ccr)_{H} sont en rapport avec l'indice de dureté Vicker (Hv)_{D} et (Hv)_{H} respectivement de sorte que (Ccr)_{D} et (Ccr)_{H} se situent entre 1,96 et 3,88 cm³/100 g tandis que (Hv)_{D} et (Hv)_{H} se situent de façon correspondante entre 300 et 500.

## Patentansprüche

1. Verfahren für die Niedertemperatur-Wärmebehandlung nach dem Schweißen (PWHT) beim Mehrschichtschweißen, mit den Stufen: Bestimmung der Restwasserstoffkonzentration Co (cc/100 g) direkt unter der letzten Schweißschicht sofort nach der Beendigung des Schweißens, Bestimmung einer rißverhindernden kritischen Wasserstoffkonzentration Ccr (cc/100 g) zur Bildung eines Verhältnisses Ccr/Co, Bestimmung des Werts eines Produkts Dₚ·tₚ aus einem Wasserstoffdiffusionskoeffizienten Dp (cm²/sek.) während der Wärmebehandlung und einer Hallezeit tp (sek.), wobei eine momentan erreichte Wasserstoffkonzentration C (cc/100 g) gleich der kritischen Wasserstoffkonzentration Ccr wird, auf der Basis der Beziehung eines Verhältnisses C/Co der momentanen Wasserstoffkonzentration C (cc/100 g) zur Restwasserstoffkonzentration Co und einer Summe eines Parameters _{T} (cm²) der Wasserstoffdiffusion gemäß der nachstehend gegebenen Formel und des Produkts Dₚ·tₚ, Messung der Temperatur der Wärmebehandlung an einer geeigneten Stelle der Schweißung, Beendigung der Wärmebehandlung zu einem Zeitpunkt, an dem ein zeitintegrierter Wert eines Wassersₜoffdiffusionskoeffizienten D_{Pi} (cm²/sek.) bei der gemessenen Temperatur den Wert von Dₚ·tₚ bei gegebenen. Bedingungen übersteigt, wobei PWHT Wärmebehandlung nach dem Schweißen bedeutet, wobei D, ein Wasserstoffdifussionskoeffizient (cm²/sek.) in einem willkürlichen Schweißabschnitt während der Schweißung jeder einheitlichen Schicht, und tn die für die Schweißung jeder einheitlichen Schicht erforderliche Zeit (Sekunde) ist, und wobei die kritische Wasserstoffkonzentration (Ccr) so auf die Zahl der Vickers-Härte (Hv) bezogen ist, daß (Ccr) im Bereich von 1,96 bis 3,88 cc/100 g liegt, während (Hv) entsprechend im Bereich von 300 bis 500 liegt.

2. Verfahren für die Niedertemperatur-PWHT nach Anspruch 1, umfassend die Bestimmung des Parameters τ der Wasserstoffdiffusion und der gelösten Wasserstoffkonzentration Co,o (cc/100 g) bei gegebenen Schweißbedingungen, und Bestimmung von Co auf der Basis der Beziehung zwischen dem Parameter τ und Co/Co,o.

3. Verfahren für die Niedertemperatur-PWHT nach Anspruch 1 oder 2, umfassend die Erwärmung einer Umfangsschweißung eines gedrehten schweren dicken Kessels mit mehr als einem Brenner, Messung der Temperatur der Schweißung an einem willkürlichen Punkt, um Änderungen eines Wasserstoffdiffusionskoeffizienten Dpⱼ mit der Zeit zu erhalten, und Ermittlung des Zeitpunktes, wenn der integrierte Zeitwert des Koeffizienten D_{Pi} den Wert von D_{P}·tₚ übersteigt.

4. Verfahren für die Niedertemperatur-PWHT nach Anspruch 1 oder 2, umfassend die Erwärmung einer Stumpfnahtlinie von einer Seite ber mittels einer Vielzahl von feststehenden Brennern während der Messung der Temperaturen an willkürlichen verschiedenen Punkten an der anderen Seite der Schweißlinie, um die Änderung des Wasserstoffdiffusionskoeffizienten D_{Pi} mit der Zeit zu erhalten, und Ermittlung eines Zeitpunktes, an dem der über die zeitintegrierte Wert von Dₚᵢ den Wert von Dₚ·t_{P} übersteigt.

5. Verfahren für die Niedertemperatur-Wärmebehandlung nach dem Schweißen bei der Mehrschichtschweißung umfaßt die Stufen: Beschaffung der Restwasserstoffkonzentration (Co)_{D} und (Co)_{H} (cc/100 g) direkt unter der zuletzt geschweißten Schicht sofort nach der Beendigung der Mehrschichtschweißung, wobei (Co)_{D} und (Co)_{H} für geschweißtes Metall (abgelargertes Metall) bzw. für den wärmebeeinflußten Bereich stehen, Beschaffung der kritischen Wasserstoffkonzentration zur Verhinderung des Schweißnahtrisses (Ccr)_{D} und (Ccr)_{H} für das geschweißte Metall bzw. für den wärmebeeinflußten Bereich, der von der maximalen Restspannung und der maximalen Vickers-Härte der Mikrostruktur im geschweißten Bereich abhängt, Beschaffung der Werte von (Ccr/Co)_{D} und (Ccr/Co)_{H}, des Verhältnisses der kritischen Wasserstoffkonzentration (Ccr)_{D} und (Ccr)_{H} zur Vermeidung eines Schweißnahtrisses sowohl in dem geschweißten Metall als auch dem wärmebeeinflußten Bereich zur Restwasserstoffkonzentration (Co)_{D} und (Co)_{H}, Beschaffung der Werte von (C/Co)_{D} und (C/Co)_{H} für das geschweißte Metall und für den wärmebeeinflußten Bereich, des Verhältnisses der Sauerstoffkonzentrationen in der geschweißten Zone (C)_{D} und (C)_{H}, die durch die Niedertemperatur-Wärmebehandlung nach dem Schweißen herabgesetzt sind, zur Restwasserstoffkonzentration (Co)_{D} und (Co)_{H}, Beschaffung der Werte von (τ + Dₚ·tₚ)_{D} und (τ +Dₚ·tₚ)_{H} für das geschweißte Metall und für den wärmebeeinflußten Bereich, wobei D_{D} der Wasserstoffdiffusionskoeffizient während der Wärmebehandlung nach dem Schweißen und tₚ die Haltezeit ist, und wobei τ (cm²) ein Wasserstoffdiffusionsparameter bei einer Schweißung unter gegebenen Bedingungen ist, wobei D, ein Wasserstoffdiffusionskoeffizient (cm²/sek.) in einer willkürlichen Schweißzone jeder einheitlichen Schicht und tn die für die Schweißung jeder einheitlichen Schicht erforderliche Zeit ist, Bestimmung des größeren Wertes (Dₚ·tₚ) aus (Dₚ·tₚ)_{D} und (Dₚ·tₚ)_{H} durch Vergleich dieser Werte als eine Bedingung für die Wärmebehandlung nach dem Schweißen, Messung der Temperatur an einem geeigneten Abschnitt der Schweißung während der Wärmebehandlung nach der Schweißung, Beeindigung der Wärmebehandlung zu einem Zeitpunkt, an dem der über die Zeit integrierte Wert des Wasserstoffdiffusionskoeffizienten (Dₚᵢ) (cm²/sek.) bei der gemessenen Temperatur den Wert von (Dₚ·tₚ) übersteigt, und wobei die kritischen Wasserstoffkonzentrationen (Ccr)p und (Ccr)_{H} so auf die Zahl der Vickers-Härte (Hv)_{D} und (Hv)_{H} bezogen sind, daß (Ccr)_{D} und (Ccr)_{H} im Bereich von 1,96 bis 3,88 cc/100 g liegen, während (Hv)_{D} und (Hv)_{H} entsprechend im Bereich von 300 bis 500 liegen.

6. Verfahren für die Niedertemperatur-PWHT einer Mehrschichtschweißung, gekennzeichnet durch die Stufen: Bestimmung der Restwasserstoffkonzentration Co (cc/100 g) für eine der Mehrschichtschweißung ähnliche Testschweißung direkt unter der zuletzt geschweißten Schicht sofort nach der Beendigung der Schweißung, Bestimmung einer rißverhindernden kritischen Wasserstoffkonzentration Ccr (cc/100 g) für die Testschweißung zur Bildung eines Verhältnisses Ccr/Co, Bestimmung des Werts eines Produkts Dₚ·tₚ aus einem Wasserstoffdiffusionskoeffizienten Dₚ (cm²/sek.) während der Wärmebehandlung und einer Haltezeit t_{c} (sek.) für die Testnaht, wobei eine momentan erreichte Wasserstoffkonzentration C (cc/100 g) gleich der kritischen Wasserstoffkonzentration Ccr wird, auf der Basis der Beziehung eines Verhältnisses C/Co der momentanen Wasserstoffkonzentration C (cc/100 g) zur Restwasserstoffkonzentration Co und einer Summe aus einem Parameter τ (cm²) der Wasserstoffdiffusion gemäß der nachstehenden Formel und des Produkts Dₚ·tₚ, Messung der Temperatur der Wärmebehandlung an einer geeigneten Stelle der Mehrschichtschweißung, Beendigung der Wärmebehandlung der Mehrschichtschweißung zu einem Zeitpunkt, an dem ein zeitintegrierter Wert des zuvor bestimmten Wassersₜoffdiffusionskoeffizienten Dₚᵢ (cm²/sek.) bei der gemessenen Temperatur den zuvor bestimmten Wert von Dp.tp übersteigt, wobei gilt wobei PWHT Wärmebehandlung nach dem Schweißen bedeutet, Dᵢ ein Wasserstoffdiffusionskoeffizient (cm²/sek.) in einem willkürlichen Schweißungsabschnitt während der Schweißung jeder einheitlichen Schicht, und tn die für die Schweißung jeder einheitlichen Schicht erforderliche Zeit (Sekunden) ist, und wobei die kritische Wasserstoffkonzentration (Ccr) so auf die Zahl der Vickers-Härte (Hv) bezogen ist, daß (Ccr) im Bereich von 1,96 bis 3,88 cc/100 g liegt, während (Hv) ensprechend im Bereich von 300 bis 500 liegt.

7. Verfahren für die Niedertemperatur-Wärmebehandlung nach dem Schweißen einer Mehrschichtschweißung, gekennzeichnet durch die Stufen: Beschaffung der Wasserstoffkonzentration (Co)c und (Co)_{H} (cc/100 g) für eine der Mehrschichtschweißung ähnliche Testschweißung direkt unter der zuletzt geschweißten Schicht sofort nach Beendigung der Mehrschichtschweißung, wobei (Co)_{D} und (Co)_{H} für geschweißtes Metall (abgelagertes Metall) bzw. für den wärmebeeinflußten Bereich stehen, Beschaffung der kritischen Wasserstoffkonzentration für die Testschweißung zur Vermeidung eines Schweißnahtrisses (Ccr)_{D} und (Ccr)_{H} für das geschweißte Metall bzw. für den wärmebeeinflußten Bereich, der von der maximalen Restspannung und maximalen Vickers-Härte der Mikrostruktur in der Schweißzone abhängt, Beschauffung der Werte von (Ccr/Co)_{D} und (Ccr/Co)_{H}, des Verhältnisses der kritischen Wasserstoffkonzentration (Ccr)_{D} und (Ccr)_{H} zur Vermeidung eines Schweißnahtrisses sowohl im geschweißten Metall als auch im wärmebeeinflußten Bereich zur Restwasserstoffkonzentration (Co)_{c} und (Co)_{H} für die Testschweißung, Beschaffung der Werte für die Testschweißung von (C/Co)_{D} und (C/Co)_{H} für das geschweißte Metall und für den wärmebeeinflußten Bereich, der Verhältnisse der Wasserstoffkonzentration in der geschweißte Zone und dem wärmebeeinflußten Bereich (C)_{D} und (C)_{H}, die durch die Niedertemperatur-Wärmebehandlung nach der Schweißung verringert sind, zur Restwasserstoffkonzentration (Co)_{D} und (Co)_{H}, für die Testschweißung Beschaffung der Werte von (τ + Dₚ·tₚ)_{D} und (τ + Dₚ·tₚ)_{H} für das geschweißte Metall und den wärmebeeinflußten Bereich, wobei Dₚ der Wasserstoffdiffusionskoeffizient während der Wärmebehandlung nach der Schweißung und tp die Haltezeit ist, und wobei τ (cm²) ein Wasserstoffdiffusionsparameter bei einer Schweißung unter gegebenen Bedingungen. ist, worin Dᵢ ein Wasserstoffdiffusionskoeffizient (cm²/sek.) in einer willkürlichen Schweißzone jeder Einheit und tn die für schweißung jeder einheitlichen Schicht erforderliche Zeit ist, Bestimmung eines Wertes (Dₚ·tₚ) für die Testschweißung, der dem größeren der Wert (Dₚ·tₚ)_{D} und (Dₚ·tₚ)_{H} aus dem Vergleich dieser Werte entspricht, als eine Bedingung für die Wärmebehandlung nach der Schweißung, Messung der Temperatur an einem geeigneten Abschnitt der Mehrschichtschweißung während der Wärmebehandlung nach der Schweißung, Beendigung der Wärmebehandlung der Mehrschichtschweißung zu einem Zeitpunkt, wenn der zeitintegrierte Wert des zuvor bestimmten Wasserstoffdiffusionskoeffizienten (Dₚᵢ) (cm²/sek.) bei der gemessenen Temperatur den zuvor bestimmten Wert von (Dₚ·tₚ) übersteigt, und wobei die kritischen Wassersₜoffkonzentrationen (Ccr)_{D} und (Ccr)_{H} auf die Zahl der Vickers-Härte (Hv)_{D} bzw. (Hv)_{H} so bezogen sind, daß (Ccr)_{D} und (Ccr)_{H} im Bereich von 1,96 bis 3,88 cc/100 g liegen, während (Hv)_{D} und (Hv)_{H} entsprechend im Bereich von 300 bis 500 liegen.
